

May 14, 1946.

R. C. WHITMAN  
RESIN-IMPREGNATED WOVEN TEXTILE FABRIC  
AND METHOD OF PRODUCING THE SAME  
Filed Sept. 15, 1944

2,400,379



Fig. 1.



Fig. 2.

Ross C. Whitman

INVENTOR.

BY Thacher H. Thach  
Attorney

## UNITED STATES PATENT OFFICE

2,400,379

RESIN-IMPREGNATED WOVEN TEXTILE  
FABRIC AND METHOD OF PRODUCING  
THE SAMERoss C. Whitman, Walpole, Mass., assignor to  
The Kendall Company, Boston, Mass., a corporation of Massachusetts

Application September 15, 1944, Serial No. 554,279

12 Claims. (Cl. 28—74)

This invention relates to resin-impregnated woven textile fabrics and methods of making the same, and the object of the invention is to provide improved fabrics of this type having moisture-resistant stiffness and which have substantially no tendency to curl. The principal commercial applications of the invention are found in the field of mechanical or industrial fabrics, particularly fabrics which may be subject to conditions of high humidity and temperature, for example, radio spiders. The fabrics hereof are also useful for condenser and insulating cloths, interlinings, hat materials, shoe linings, and laminated fabrics commonly made from muslins, drills, twills, and sheeting materials. Resin-impregnated fabrics as heretofore known and used in the art have curled to a substantial extent and the present invention provides a satisfactory and certain basis for substantially eliminating such objectionable curling during not only cutting and fabrication into various articles of manufacture (which is sufficient for many purposes) but also during the utilization thereof, for example, fabrics which must retain a certain stiffness even where subject to severe atmospheric conditions of heat and moisture.

The present invention provides novel resin-impregnated fabrics in which undesirable curl is overcome and this latter condition is maintained despite atmospheric changes and provides a ready method of producing such fabrics without the use of special equipment and without substantial increase in manufacturing cost. In accordance with my inventions as more fully described in my co-pending applications, Serial Numbers 512,211 and 525,719, filed November 11, 1943, and March 9, 1944, respectively, the factors which influence fabric curl in stiffened fabrics are yarn size of component yarns as the major factor and, as other factors, direction and degree of yarn twist, and the number of yarn ends per inch of fabric in the warp and filling directions. Also, as set forth in said applications, the sets of warp and filling yarns have a profound relationship and effect inter se and the fabric curling or torque effect exerted by a given warp yarn can be and is neutralized or offset by the curling effect of a filling yarn of the same size and the same twist (same number of turns per inch and same direction of twist), and, further, the curling effect of one set of yarns (warp or filling) can be neutralized by the other set of yarns whether of unidirectional twist or whether including yarns of both directions of twist, and though said other set also differs from the first

5 set in yarn size, in twist multiple, and in number of yarns per inch of fabric, the difference occurring in two or more of the factors. The method of practicing the present invention by incorporating my said discoveries in the manufacture of resin-impregnated moisture-resistant fabrics having substantially no tendency to curl is fully set forth hereinafter.

Study of certain stiffened fabrics, including the 10 resin-impregnated cellulosic fabrics of this invention, resulted in the paradoxical discovery that in such fabrics the curl is caused by an increase in the twist (i. e., a twisting tighter) of the dominant component yarns, these yarns imparting a net curling effect even though the same set of yarns include stiffened yarns of opposite twist. For example, when a foot square piece of a certain commercial resin-impregnated fabric was laid upon a flat surface, it was observed 15 to curl in that two of the diagonal corners lifted up somewhat from the flat surface and the other two diagonal corners attempted to curl downwardly. The curl here was caused by a twisting tighter of certain component yarns.

20 25 By properly applying these discoveries in yarn manufacture and selection, in weave layout and weaving of textile fabrics for resin impregnation, one can produce a wide range of novel resin-impregnated stiffened moisture-resistant fabrics 30 (with warp and filling of the same or opposite directions of twist) which are characterized by a substantial absence of curl even though resin-impregnated and by a moisture resistance such that the fabric retains a high stiffness even when 35 thoroughly wetted.

In the drawing, showing preferred types of fabrics of this invention,

Fig. 1 is an enlarged diagrammatic view illustrating a resin-impregnated square weave fabric 40 of unidirectional twist; and

Fig. 2 is a diagrammatic view illustrating a resin-impregnated fabric wherein one set of yarns is unidirectional and the other set includes yarns of opposite direction of twist.

45 Referring to the drawing in which like numerals represent like parts, Fig. 1 illustrates a non-curling resin-impregnated fabric of this invention with cellulosic Z-twist warp yarns 2 of smaller size than the cellulosic filling yarns 3 with the 50 latter equal in number of ends but of lower degree (not shown) of unidirectional Z-twist, in which both sets of yarns tend to twist tighter because of their resin-impregnation, the tendency of the warp yarns 2 to lift the diagonal opposite lower and upper corners of the fabric, as oriented

in the drawing, being neutralized by the filling yarns 3 so that the corners all lie flat and the fabric does not curl.

Fig. 2 shows another example of resin-impregnated non-curling fabric of this invention with cellulosic warp yarns 4—Z and 4—S of opposing twists, there being five yarns 4—Z for each yarn 4—S as shown. These warp yarns are of larger size than the unidirectional Z-twist cellulosic filling yarns 5, with the latter equal in number of ends with the required degree of twist (not shown) in which both sets of yarns tend to twist tighter because of the resin-impregnation, the net tendency of the warp yarns to lift the lower and upper corners being neutralized by the set of filling yarns so that the corners of the fabric all lie flat and the fabric does not curl despite the resin-impregnation.

Nearly all woven textile fabrics have as many or more warp yarns than filling yarns so that, from the standpoint of end count, most (but not all) typical applications of the invention fall in between a square weave fabric, with its equal number of ends per inch of warp and filling yarns, and a fabric with a two-to-one or higher ratio of warp to filling ends per inch, though the invention is also applicable to fabrics wherein the number of filling ends per inch exceeds that of the warp. Also, for similar reasons of economical and practical manufacture on modern spinning and weaving equipment, nearly all fabrics heretofore, particularly industrial fabrics, have larger warp yarns than filling yarns. For the same reasons, warp twist has been almost invariably higher than filling twist, in the trade, "warp twist" is synonymous with high twist, and "filling twist" is synonymous with low twist.

The foregoing principles of the invention afforded a basis for my derivation of a mathematical equation which, as a practical matter, gives a general guide for successful application and use of the invention in the actual manufacture of the resin-impregnated non-curling fabrics of this invention. The basic equation is as follows:

$$\frac{\left(M_w - \frac{N_w}{66}\right)E_w}{\sqrt{N_w^3}} = \frac{\left(M_f - \frac{N_f}{66}\right)E_f}{\sqrt{N_f^3}}$$

where

M is twist multiple,  
N is yarns number (size),

E is end count, and

w and f refer to warp and filling, respectively.

In the use of the equation for fabric design and manufacture after the general construction as to end count and yarn size has been determined, the equation is applied first only to warp and filling yarns of unidirectional twist whether the fabric be simply unidirectional or whether it have unidirectional yarns in but one of the two sets of yarns. If the latter type, the equation is applied first to the unidirectional set of yarns (whether such set be filling, as usually preferred, or warp) and to the yarns of the same direction of twist in the other or second set and to solve the equation so as to determine the number of such latter yarns necessary to neutralize the fabric curling tendency of the first set. The remaining yarns of said second set are then divided equally into yarns of each direction of twist (it being assumed that all the yarns of said second set are of the same size and twist multiple). Referring to the fabric of Fig. 2, for example, the equation is first applied to filling yarns of uni-

directional Z-twist and the required number of warp yarns of the desired size of the same direction of twist necessary to neutralize the fabric curling tendency of said filling yarns is determined, here four warps per six fillings. This leaves two warp yarns for each basic unit of this fabric construction, which two warp yarns are then divided into 1—S and 1—Z, all of the warp yarns in this example being of the same size and twist multiple. This gives the square weave fabric as shown in Fig. 2 in which there are six Z-twist filling yarns for six warp yarns made up of five Z-twist yarns and one S-twist yarn.

Normally, as in the preferred fabrics of this invention, at least one set of yarns is of unidirectional twist, and in the majority of cases where but one set is unidirectional, the filling set is of unidirectional twist, rather than the warp set, for, in such cases, the warp set normally and conventionally would be the dominant set to be modified in accordance with this invention. If the filling set includes yarns of opposite twist, important economic advantages are lost, particularly where box looms would be required to insert singles yarns of opposite twist. Though both sets may include yarns of opposing twist, it is not necessary, and, similarly, important advantages are lost in so doing.

Where each set includes yarns of opposing twist (as well as where but one set does), the basic equation may be applied to give the net fabric curling effect of each set as follows:

$$35 \left[ \frac{\left(M_w - \frac{N_w}{66}\right)E_w}{\sqrt{N_w^3}} \right]_s + \left[ \frac{\left(M_f - \frac{N_f}{66}\right)E_f}{\sqrt{N_f^3}} \right]_s = \left[ \frac{\left(M_w - \frac{N_w}{66}\right)E_w}{\sqrt{N_w^3}} \right]_s + \left[ \frac{\left(M_f - \frac{N_f}{66}\right)E_f}{\sqrt{N_f^3}} \right]_s$$

where M equals twist multiple, N equals yarns number, E equals end count, w and f refer to warp and filling respectively, and Z and S refer to the respective directions of twist.

45 If either set of yarns includes yarns differing from each other in size or twist multiple, it will be necessary to consider each group of similar yarns separately and add together the results thereof to obtain the total net factor for each set.

50 The twist multiple employed in this equation is the same as that employed in the textile art and equals twist turns per inch of yarn divided by the square root of the yarn number (cotton system), and for the purpose of the equation, and in the specification and claims, the size of all yarns is expressed on the cotton system, for example, 350 denier rayon yarns are classified approximately as number 15.2; and the expression "end count" is to be taken as meaning the number of yarns per inch of fabric in the designated direction. In the application and use of the invention, it is not necessary strictly to adhere to absolute equality as variations from the equality represented by the equation are necessarily encountered in practice, the ultimate test being whether any given fabric embodies the principles and features of the invention as herein described and claimed.

70 In accordance with this invention, there is applied to the original fabric water or solvent-carried potentially water-insoluble resin or resin-forming materials. Various resins such as phenol formaldehyde, urea formaldehyde, melamine formaldehyde, protein (e. g. casein) formaldehyde, polystyrene, the alkyd resins, and the methacrylates may be used for this purpose. Since

these resin materials are water-insoluble when applied, or are rendered water-insoluble after application (by baking the impregnated fabric, usually), the stiffness obtained is not immediately or readily removed when the fabric is washed. The determining factor in the choice of the resin and its method of application is that water must be present during the polymerization of the resin and the consequent stiffening of the fabric. This water may be formed as a product of the condensation of the resin or may be present in the liquid impregnating mixture as a solvent or a carrier.

The impregnating materials should be applied in sufficient quantity and concentration so that the resultant end product includes 20 to 150% by weight of resin (based on the weight of the fabric) in order to provide the desired moisture-resistant properties. In the preferred practice of this invention, when thoroughly wetted, for example, for 15 minutes in water at 70° F., the fabric possesses a stiffness of more than 50% of its stiffness at 32% relative humidity at the same temperature. This corresponds with a piece of fabric at an ordinary outdoor temperature, being very dry, as compared with being subject to extremes of humidity or moisture. This is a typical condition encountered in radio loud speakers, e. g., at sea or under tropical conditions under which the resin-impregnated fabric membrane must maintain substantially its original degree of stiffness measured immediately after the resin has been cured or polymerized. Such stiffness may be conveniently expressed in units of mean flexural rigidity (milligram centimeters) as incident to a standard Pierce Flexometer, and the same typical fabrics with their weights and stiffness are as follows:

#### Example 1

A heavy stiffened fabric used for stamping out the crown and brim of men's summer hats was found to have objectionable curling characteristics, which not only made the cutting operation difficult, but also gave the brim an uneven roll. This base fabric had an actual end count of 20.1 x 17.9 with 3 1/2's yarns in the warp and 4's in the filling, the corresponding twist multiples being 4.25 and 3.27. By altering the specifications so that the yarn weights were 3.98 in the warp and 3.19 in the filling, and keeping the same end count and filling twist multiple, it was found by solving the equation for the warp twist multiple that the value of 4.07 would give a fabric with a warp preponderance of only .003. This fabric when resin-impregnated according to the teaching of this application exhibited no tendency to curl, and showed exceptional resistance to moisture. The average flexural rigidity of warp and filling when measured at 70° F. and 32% relative humidity was 45,000, when the resin content based on the weight of the fabric was 35%. After soaking the sample in water at the same temperature for fifteen minutes, there was no apparent loss in stiffness.

#### Example 2

A non-curling resin impregnated batiste with an end count of approximately 88 x 80 was found to retain 57% of the stiffness measured at 70° F. and 32% relative humidity after it had been soaked for fifteen minutes in water at 70° F. This fabric had a resin content of 98% based on the weight of the untreated fabric and the flexural rigidity measured under the initially stated con-

dition was 2300. In setting up the specifications for this fabric so that a non-curling cloth would result, it was found that the method of balancing employed in the previous example could not be used here. The yarn weights in this fabric are 69.91's in the warp and 95.32's in the filling. Substituting these along with the actual end count of 87.6 x 79.3 and the twist multiples of 5.56 in the warp and 5.12 in the filling in the formula gives a filling value of .3136, compared with a warp value of .7298. In order to bring these values close enough to produce a non-curling fabric, the yarn numbers and other values would have to be very considerably changed. Rather than do this, the fabric may be balanced by using both S and Z yarns in the warp and only Z yarns in the filling. The ratio of S and Z yarns in the warp may be found in the following way, the number of ends per inch of Z twist yarn required in the warp to exactly balance the filling will be found by setting the warp side of the equation equal to the filling value which has already been found and solving for E. This is found in this case to be 40.7 ends per inch. Subtracting 40.7 from 87.6, the total warp count gives 46.9 ends per inch which must be balanced and therefore equally divided between S and Z twist yarns. This means that there should be 23.45 ends per inch of S twist yarn and 64.15 ends per inch of Z twist yarn. Such a ratio may be approximated by tying three Z twist yarns to every one S twist yarn in the warp of our fabric. By this arrangement the warp value is changed to .3372 and the fabric is out of balance by .024 unit which gives a substantially non-curling fabric.

#### Example 3

A radio spider which lies flat may be stamped from a resin impregnated non-curling 64 x 60 fabric. This fabric which has an actual end count of 63.8 x 59.0 with 29.81's yarns in the warp and 29.92's yarns in the filling may be balanced by properly adjusting the twist multiples. If the warp twist multiple is taken as 4.10, the warp value calculates to be 1.431. If the filling is then given a twist multiple of 4.31, the filling formula value is 1.392 and the warp preponderance is only .039 which is low enough to give a balanced non-curling fabric. The flexural rigidity of this fabric when impregnated with a phenol formaldehyde solution so that the resin content based on the weight of the base fabric is 60%, is 7,500 measured at 70° F. and 32% relative humidity. After soaking in water in the same test applied in the previous examples, 60% of the stiffness is retained.

#### Example 4

A 70 x 40 drill suitable for use as a shoe lining may be treated with a resin so that the resin content of the fabric will be 29% based on the weight of the untreated fabric, and the flexural rigidity measured under the usual conditions, that is, 70° F. and 32% relative humidity, will be 400. Virtually all of this stiffness is retained even after the usual soaking treatment. Freedom of this fabric from curl may be assured by setting up the specifications for weaving according to the formula. Calculation of the warp and filling values for an ordinary non-balanced fabric of this type gives 6.091 and 2.046, respectively, indicating that balance will be difficult to achieve using yarn of only one direction twist and changing slightly the given specifications. For this reason, it was decided to weave the sample with alternate 75 S and Z yarns in the warp. Using this same

filling value, calculated from the filling specification of 38.9 ends per inch with 15.95's yarns with a twist multiple of 3.59, we find that 23.3 ends of 13.48's warp yarns with a twist multiple of 4.55 are needed to balance the filling. Since the desired number of ends per inch in the warp is actually 69.3, the difference must be equally divided between S and Z yarns. A tie-in of one S yarn to two Z yarns in the warp will approximately accomplish this, giving a fabric which has a filling preponderance of .016 and which is therefore essentially non-curling.

*Example 5*

A heavy 52 x 36 duck, resin-treated to give it a moisture-resistant stiff finish, may be made to lie flat by making it according to the following specifications. The original fabric had an actual end count of 51.6 x 35.8 and calls for the use in the warp of 9.03's yarns with a twist multiple of 4.01 and in the filling of 11.52's yarns with a twist multiple of 3.46. These values will give a warp figure of 7.359 and a filling value of 3.012 which indicates that the fabric is way out of balance and that the more satisfactory way of making it non-curling requires the use of oppositely twisted yarns in the warp. Using the given filling value and the yarn number and twist multiple of the warp yarns, it is found that 21.1 ends per inch are required to balance the filling. If the rest of the 30 yarns are equally divided between S and Z twist, there will be 36.35 ends per inch of Z twist yarn and 15.25 ends per inch of S twist yarn, which is found to correspond quite closely to a ratio of two S twist yarns to five Z twist yarns. With this warp tie-in, the fabric is found to have a warp preponderance of .142 which is sufficiently small to give a non-curling fabric. The resin treatment accorded this fabric which consisted of the application of enough resin solution so that the resin content of the finished fabric was 60% based on the weight of the untreated cloth, resulted in the fabric exhibiting a flexural rigidity of 365,000 at 70° F. and 32% relative humidity. After soaking in water at 70° F. for fifteen minutes, this resin-impregnated duck retained 62% of its original stiffness.

*Example 6*

A non-curling viscose cotton blend (60% viscose and 40% cotton) may be given a moisture-resistant stiff finish by treating it with a melamine formaldehyde resin so that the resin content of the stiffened fabric is 53% based on the weight of the untreated cloth. This fabric has a flexural rigidity of 34,000 when measured at 32% relative humidity and 70° F. and 70% of this stiffness is retained after the fabric has undergone the soaking treatment described in the previous examples. This fabric has an actual end count of 43.9 by 41.5 and has 14.87's yarns in the warp and 12.11's yarns in the filling. It was found that the fabric could be balanced without resorting to the use of oppositely twisted yarns in the warp by suitably adjusting the twist multiples. A twist multiple of 4.47 in the warp and of 3.40 in the filling will give warp and filling values such that the warp preponderance will be .076. Because of this low value, the fabric embodying these specifications will lie flat.

*Example 7*

A stiffened condenser fabric which is resistant to moisture and which will not curl under any

condition may be made by treating a 76 x 72 lawn with a melamine formaldehyde resin so that the resin content is 90% based on the weight of the untreated fabric. The flexural rigidity of this fabric, the specifications for which are given below, is 1,300 when measured under the usual conditions, and only 20% less when measured after the fabric has been soaked in water for fifteen minutes at 70° F. In order that the fabric be non-curling, the specifications are set up in accordance with the equation for balanced fabrics. When the end count, yarn numbers, and twist multiples, 75.8 x 71.3; 59.52's, 85.41's; 4.45, 3.39, respectively, for a standard fabric of this type are substituted in the equation, it is seen the warp value is .5860 and the filling value .1897. This is, of course, far from a non-curling fabric. Because it is desirable to keep essentially the appearance and characteristics of this fabric, however, it seemed advisable to balance this fabric by using alternate S and Z yarns in the warp. By carrying out similar calculations to those used in Example 2, it was discovered that a warp tie-in of one S yarn to every two Z yarns would give a fabric with a warp preponderance of only .005, and consequently a non-curling fabric.

The resins may be applied to fabrics made of any type of cellulosic or predominantly cellulosic textile fabrics plain or mixed or to plain or mixed yarns including staple or cut staple natural or synthetic cellulosic fibers, or continuous cellulosic filaments (later referred to). Though non-cellulosic synthetic or natural fibres or filaments may be included in minor proportions, it must be borne in mind that in none of these non-cellulosic fibres does a water-swelling and stiffening with resultant reversal of curl occur, as in the predominant cellulosic fibres.

The preferred impregnated fabrics of this invention are made from fabrics woven from or including yarns made up of, or which include predominantly cotton or other natural cellulosic fibres such as sisal, ramie, hemp or jute, or synthetic cellulosic fibres such as viscose, cuprammonium and other regenerated cellulosic fibres (either cut staple or continuous filament).

Various impregnated fabrics may be made which include a substantial proportion of yarns in the warp, filling, or both, which are not swollen and stiffened so as to produce a reverse curl (yarns twisting tighter), in such fabrics the warp and filling each including swollen and stiffened yarns with their reverse fabric curling tendencies offset in general accordance with the foregoing disclosure. In such cases the curling effect of the proportion of yarns not producing reverse curl may be safely disregarded as not significant in view of their relatively negligible effect upon curling as compared with that of the pronounced and very much greater curling effect of the swollen and stiffened warp and filling yarns producing reverse curl.

In the practice of this invention, it is important to provide warp yarns and filling yarns 65 that are spun with precision from uniform card sliver to definite sizes and twist multiples, and so woven that all areas of the body of the fabric are strictly uniform in construction since it is these factors, and their relation to each other, 70 that are depended upon in arriving at the desired result. Even with the most modern equipment, and with carefully controlled spinning-room humidity, it is well known that considerable variation in the yarn size occurs as spinning proceeds. A spinning machine balanced and ad-

Justed to produce 30's yarns may, after a week or ten days' operation, be found to be delivering as fine as 35's or 36's, or as heavy as 27's or 26's, the shift toward lighter yarns usually proceeding faster and further than the shift towards heavier yarns. These variations are usually explained as resulting from humidity changes, temperature changes, stock changes, and machine wear, producing maladjustments.

Standard practice in modern textile mills calls for the analysis of yarns approximately every two weeks, and the readjustment of yarns size prescribed is made usually on the first roving frame, usually called the "slubber," or the second roving frame, known as the "first intermediate." This measure of control is satisfactory for ordinary fabric manufacture, but since it would permit "drifting" of yarn size to the extent mentioned above, it is obvious from the equation underlying this invention that it is entirely inadequate for the practice of the invention. Also, any change in yarn size produces a significant change in twist multiple since the spinning-frame delivers a fixed number of turns per inch to the yarn, rather than a fixed twist multiple. In the manufacture of fabrics of this invention, it is recommended that yarn analyses and equipment adjustment as needed be made daily, usually at the second drawing frame rather than on any of the succeeding roving frames. In addition, special care should be taken in the control of spinning-room humidities, etc.

In making use of the equation, actual yarn sizes, as determined by analyses in the spinning-room, and actual twist multiples, as determined by well known formulas involving spinning-frame gears, should be used rather than the "theoretical" or "standard" values. Similarly, actual end counts as reported by the weave room should be used. It is found that usually the slight changes in the end counts occasioned by variations in tension on the loom are not troublesome providing the cloth tension is checked and adjusted daily in the usual way. For fabrics where a substantially complete absence of curl is the requirement, as in radio spiders, it is found that the old style friction let-off on the loom is to be preferred to automatic positive let-off mechanism, such as the "Roper-Draper" or "Bartlett," which permit greater variations in end counts since they control tension with less precision, generally. Also, reasonable care should be taken to avoid any considerable distortion of the woven "neutralized" fabric in subsequent finishing processes. With fairly equal tensions therein so that the end count in the finished fabric is roughly equally higher or equally lower in both the warp and the filling, however, no trouble need be anticipated on this score.

The original or base fabrics utilized in the manufacture of the resin-impregnated fabrics of this invention may conveniently be tested and compared from the standpoint of curl by cutting small five-inch squares from the base fabric, impregnating such squares with a standard resin-forming solution, hot ironing the test specimens, and then noting their deformation under standard conditions, for example, by noting the rise or elevation of any corner from a horizontal supporting surface, not to exceed 1½ inches. The preferred and most searching test for base cellulosic fabrics of cotton and/or viscose rayon is by first impregnating the fabric in a solution made up as follows:

|                                                                                                                 | Parts |
|-----------------------------------------------------------------------------------------------------------------|-------|
| Bakelite solution (XR568, partially polymerized phenol formaldehyde solution, 40% Bakelite, 60% methyl alcohol) | 4     |
| Methyl alcohol                                                                                                  | 1     |
| Water                                                                                                           | 5     |

The pick-up of the solution by the base fabric may, for example, be from 125 to 150% by weight (on the weight of base fabric). The sample is then pressed between two heated metallic surfaces (net total pressure 10 lbs.) at a temperature of approximately 150° C., for sixty seconds, in order to completely polymerize and set the resin, thus forming a product of this invention. The sample is then at once removed and placed without restraint on a horizontal surface, such as a table, and promptly observed. Since this test is so searching, as a practical matter, the fabrics of this invention so made may be regarded as having substantially no tendency to curl if the sample remains substantially extended and no corner thereof rises more than 1 to 1½ inches above the supporting horizontal surface upon which it was placed. Fabrics made in accordance with the preferred practice of this invention incorporating therein any of the resins mentioned above are well within the amount mentioned. The impregnating materials hereinbefore referred to as employed in ordinary commercial use will not cause the rise of a corner of a five inch test square more than ½ to 1 inch above the supporting horizontal surface.

Having thus described my invention, what I desire to claim as new is:

35 1. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, said sets and yarns thereof being so related with respect to twist direction, twist multiple, yarns number and count as to produce substantially the equality represented by the equation

$$50 \left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

55 where M equals twist multiple, N equals yarns number, E equals end count, w and f refer to warp and filling, respectively, and Z and S refer to right and left-hand twist, respectively, thereby providing an impregnated fabric having a neutralized curling tendency and moisture-resistant stiffness characteristics.

2. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, at least one of said sets including a substantial number of yarns of each direction of twist, said sets and yarns thereof being so related with respect to twist direction, twist multi-

ple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where  $M$  equals twist multiple,  $N$  equals yarns number,  $E$  equals end count,  $w$  and  $f$  refer to warp and filling, respectively, and  $Z$  and  $S$  refer to right and left-hand twist, respectively, thereby providing an impregnated fabric having a neutralized curling tendency and moisture-resistant stiffness characteristics.

3. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, both of said sets including a substantial number of yarns of each direction of twist, said sets and yarns thereof being so related with respect to twist direction, twist multiple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where  $M$  equals twist multiple,  $N$  equals yarns number,  $E$  equals end count,  $w$  and  $f$  refer to warp and filling, respectively, and  $Z$  and  $S$  refer to right and left-hand twist, respectively, thereby providing an impregnated fabric having a neutralized curling tendency and moisture-resistant stiffness characteristics.

4. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, both of said sets having yarns of unidirectional twist, said sets and yarns thereof being so related with respect to twist direction, twist multiple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where  $M$  equals twist multiple,  $N$  equals yarns number,  $E$  equals end count,  $w$  and  $f$  refer to warp and filling, respectively, and  $Z$  and  $S$  refer to right and left-hand twist, respectively, thereby providing an impregnated fabric having a neu-

tralized curling tendency and moisture-resistant stiffness characteristics.

5. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, said set and yarns thereof being so related with respect to twist direction, twist multiple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

25 where  $M$  equals twist multiple,  $N$  equals yarns number,  $E$  equals end count,  $w$  and  $f$  refer to warp and filling, respectively, and  $Z$  and  $S$  refer to right and left-hand twist, respectively, thereby providing an impregnated fabric having a neutralized curling tendency and moisture-resistant stiffness characteristics, said fabric after wetting for 15 minutes in water at 70° F. exhibiting at least two-thirds of its stiffness in an atmosphere of 30% relative humidity at 70° F.

35 6. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, at least one of said sets including a substantial number of yarns of each direction of twist, said sets and yarns thereof being so related with respect to twist direction, twist multiple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

55 where  $M$  equals twist multiple,  $N$  equals yarns number,  $E$  equals end count,  $w$  and  $f$  refer to warp and filling, respectively, and  $Z$  and  $S$  refer to right and left-hand twist, respectively, thereby providing an impregnated fabric having a neutralized curling tendency and moisture-resistant stiffness characteristics, said fabric after wetting for 15 minutes in water at 70° F. exhibiting at least two-thirds of its stiffness in an atmosphere of 30% relative humidity at 70° F.

65 7. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns,

with the yarns of both of said sets uniformly dispersed and arranged throughout the body of the fabric, both of said sets including a substantial number of yarns of each direction of twist, said sets and yarns thereof being so related with respect to twist direction, twist multiple, yarns number and count as to produce substantially the equality represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where M equals twist multiple, N equals yarns number, E equals end count, w and f refer to warp and filling, respectively, and Z and S refer to right and left-hand twist, respectively, thereby providing an impregnated fabric having a neutralized curling tendency and moisture-resistant stiffness characteristics, said fabric after wetting for 15 minutes in water at 70° F. exhibiting at least two-thirds of its stiffness in an atmosphere of 30% relative humidity at 70° F.

8. A textile material adapted for industrial use comprising a resin-impregnated stiffened woven fabric having substantially no tendency to curl, composed essentially of sets of twisted cellulosic yarns and a resinous impregnation to at least 20% of the original base fabric weight, including a set of warp yarns and a set of filling yarns, with the yarns of both of said sets uniformly dispersed and arranged throughout the body of the fabric, both of said sets having yarns of unidirectional twist, said sets and yarns thereof being so related with respect to twist direction, twist multiple, yarns number and count as to produce substantially the quantity represented by the equation

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where M equals twist multiple, N equals yarns number, E equals end count, w and f refer to warp and filling, respectively, and Z and S refer to right and left-hand twist, respectively, thereby providing an impregnated fabric having a neutralized curling tendency and moisture-resistant stiffness characteristics, said fabric after wetting for 15 minutes in water at 70° F. exhibiting at least two-thirds of its stiffness in an atmosphere of 30% relative humidity at 70° F.

9. The method of producing a woven fabric for industrial uses having moisture-resistant stiffness characteristics and substantially no tendency to curl which consists in spinning, selecting, and weaving a set of uniform warp yarns and a set of uniform filling yarns, the warp yarns being so related to the filling yarns with respect to twist direction and multiple, yarn number and count as to produce substantially the equality represented by the equation:

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where M equals twist multiple, N equals yarns number, E equals end count, w and f refer to warp and filling respectively, and Z and S refer to the respective directions of twist, and then impregnating said fabric with a resinous medium amounting to 20 to 150% of the original base fabric weight, thereby providing an impregnated fabric having said neutralized curling tendency and moisture-resistant stiffness characteristics.

10. The method of producing a woven fabric for industrial uses having moisture-resistant stiffness characteristics and substantially no tendency to curl, which consists in spinning, selecting, and weaving a set of uniform warp yarns and a set of uniform filling yarns, at least one of said sets being of unidirectional twist, the warp yarns being so related to the filling yarns with respect to twist direction and multiple, yarn number and count as to produce substantially the equality represented by the equation:

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where M equals twist multiple, N equals yarns number, E equals end count, w and f refer to warp and filling respectively, and Z and S refer to the respective directions of twist, and then impregnating said fabric with a resinous medium amounting to 20 to 150% of the original base fabric weight, thereby providing an impregnated fabric having said neutralized curling tendency and moisture-resistant stiffness characteristics.

11. The method of producing a woven fabric for industrial uses having moisture-resistant stiffness characteristics and substantially no tendency to curl, which consists in spinning, selecting, and weaving a set of uniform warp yarns and a set of uniform filling yarns, at least one of said sets including a substantial number of yarns of each direction of twist, the warp yarns being so related to the filling yarns with respect to twist direction and multiple, yarn number and count as to produce substantially the equality represented by the equation:

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = \left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z$$

where M equals twist multiple, N equals yarns number, E equals end count, w and f refer to warp and filling respectively, and Z and S refer to the respective directions of twist, and then impregnating said fabric with a resinous medium amounting to 20 to 150% of the original base fabric weight, thereby providing an impregnated fabric having said neutralized curling tendency and moisture-resistant stiffness characteristics.

12. The method of producing a woven fabric for industrial uses having moisture-resistant stiffness characteristics and substantially no tendency to curl which consists in spinning, selecting, and weaving a set of uniform warp yarns and a set of uniform filling yarns, both of said sets including a substantial number of yarns of each direction of twist, the warp yarns being so related to the filling yarns with respect to twist direction

and multiple, yarn number and count as to produce substantially the equality represented by the equation:

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = 5$$

$$\left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z 10$$

where M equals twist multiple, N equals yarns number, E equals end count, *w* and *f* refer to warp and filling respectively, and Z and S refer to the respective directions of twist, and then impregnating said fabric with a resinous medium amounting to 20 to 150% of the original base fabric weight, thereby providing an impregnated fabric having said neutralized curling tendency and moisture-resistant stiffness characteristics.

ROSS C. WHITMAN.

### Certificate of Correction

Patent No. 2,400,379.

May 14, 1946.

ROSS C. WHITMAN

It is hereby certified that errors appear in the printed specification of the above numbered patent requiring correction as follows: Page 6, second column, line 12, claim 5, for "set" read *sets*; page 7, first column, line 39, claim 8, for "quantity" read *equality*; page 7, second column, line 17, claim 10, for "filling" read *filling*; page 8, first column, line 11, claim 12, for that portion of the formula reading

$]+[\quad \text{read} \quad ]_s + [$

and that the said Letters Patent should be read with these corrections therein that the same may conform to the record of the case in the Patent Office.

Signed and sealed this 10th day of September, A. D. 1946.

[SEAL]

LESLIE FRAZER,  
*First Assistant Commissioner of Patents.*

and multiple, yarn number and count as to produce substantially the equality represented by the equation:

$$\left[ \frac{\left( M_w - \frac{N_w}{66} \right) E_w}{\sqrt{N_w^3}} \right]_z + \left[ \frac{\left( M_f - \frac{N_f}{66} \right) E_f}{\sqrt{N_f^3}} \right]_s = 5$$

$$\left[ \frac{\left( M_w - \frac{N_w}{66} \right) E_w}{\sqrt{N_w^3}} \right]_s + \left[ \frac{\left( M_f - \frac{N_f}{66} \right) E_f}{\sqrt{N_f^3}} \right]_z 10$$

where M equals twist multiple, N equals yarns number, E equals end count, *w* and *f* refer to warp and filling respectively, and Z and S refer to the respective directions of twist, and then impregnating said fabric with a resinous medium amounting to 20 to 150% of the original base fabric weight, thereby providing an impregnated fabric having said neutralized curling tendency and moisture-resistant stiffness characteristics.

ROSS C. WHITMAN.

### Certificate of Correction

Patent No. 2,400,379.

May 14, 1946.

ROSS C. WHITMAN

It is hereby certified that errors appear in the printed specification of the above numbered patent requiring correction as follows: Page 6, second column, line 12, claim 5, for "set" read *sets*; page 7, first column, line 39, claim 8, for "quantity" read *equality*; page 7, second column, line 17, claim 10, for "filling" read *filling*; page 8, first column, line 11, claim 12, for that portion of the formula reading

$]+[\quad \text{read} \quad ]_s + [$

and that the said Letters Patent should be read with these corrections therein that the same may conform to the record of the case in the Patent Office.

Signed and sealed this 10th day of September, A. D. 1946.

[SEAL]

LESLIE FRAZER,  
*First Assistant Commissioner of Patents.*